

Sept. 27, 1932.

G. H. JACOBS

1,879,278

CARTRIDGE

Filed Sept. 1, 1931



*Fig. 3*

*Fig. 4*

*Fig. 5*



*Fig. 1*



*Fig. 2*

INVENTOR

BY

George H. Jacobs.  
Ward & Ward

ATTORNEYS

## UNITED STATES PATENT OFFICE

GEORGE H. JACOBS, OF KINGS MILLS, OHIO, ASSIGNOR TO THE PETERS CARTRIDGE COMPANY, OF KINGS MILLS, OHIO, A CORPORATION OF OHIO

## CARTRIDGE

Application filed September 1, 1931. Serial No. 560,591.

This invention relates to improvements in ammunition particularly cartridges of the type used in small arms. It is well known that cartridges are usually lubricated for storage and use with a mixture of greases having a low melting point or with an oil that is liquid at ordinary temperatures. It is also well known that due to the physical properties of the lead bullet and the metal of the shell it is practically impossible to make a tight joint between the shell and the bullet by crimping which is the usual method of connection. Thus it frequently happens that the cartridges are damaged or rendered useless because of the penetration of the lubricant into the powder and priming charge of the shell by way of the crevice or joint between the bullet and shell. This penetration to powder and priming charge may also occur about the priming cup in the instance of center-fire cartridges in which case the damage more immediately and directly occurs to the priming charge.

It is, therefore, the object of this invention to provide a cartridge which is sealed against the entrance of moisture, oils, greases, and corrosive vapors and gases and to provide an improved and highly suitable grease or oil-proof compound, the sealing material being efficiently applied at the juncture of the bullet and shell and about the priming cup.

Cartridges which have been sealed may be stored in the chamber of the gun or in the magazine which may be liberally supplied with oil without danger of the oil seeping into and saturating the powder and thereby deteriorating the cartridge. Likewise cartridges, which have been sealed and then lubricated with a wax or grease having a low melting point, may be stored at temperatures in excess of the melting point of the lubricant in view of the fact that even though the lubricant becomes liquid and mobile, there is no opportunity for the lubricant to creep into the cartridge.

Other objects and certain advantages will be more fully apparent from a description of the accompanying drawing, in which:

Figure 1 is a longitudinal sectional view of a cartridge of the center-fire type showing

the sealing material applied at the joint of bullet and shell and applied at the priming cup.

Figure 2 is a bottom plan view of the sealed rim-fire cartridge.

Figure 3 is a longitudinal sectional view of a rim-fire cartridge showing the sealing material applied at the joint of shell and bullet.

Figure 4 is a side view of a cartridge shown partly in section with the bullet detached for illustrating the sealing material applied initially to the shell.

Figure 5 is a view taken similar to Figure 4 but showing the sealing material initially applied to the heel of the bullet.

Referring to the drawing, the shell is indicated at 10 and the bullet at 11. In the instance of the center-fire cartridge as shown in Figures 1 and 2, a priming cup 12 is secured in a recess in the center at the underside of the shell and an aperture 13 affords communication and contact between the priming mixture and the powder 14. The powder charge fills the shell with the exception of a space for the heel 15 of the bullet. For the purpose of attachment of the bullet to the shell, an annular groove 16 is provided in the bullet and the upper edge of the shell is crimped or clinched into this recess.

The sealing compound is applied as at 17 to the joint between shell and bullet and fills the recess. This application of the sealing compound after the shell is loaded is preferable. The sealing compound is applied as at 18 about the priming cup filling or closing the lower end of the pocket or recess containing the priming cup.

In the instance of the rim-fire cartridge as shown in Figures 3, 4 and 5, the priming mixture 19 is contained at the base of the shell within the rim portion 20 and no sealing is necessary at this point. For the purpose of receiving the clinched or crimped upper edge of the shell for attachment purposes, the annular groove 16 is included in the bullet beneath the shoulder 21 of the bullet.

In this instance the sealing compound is shown applied in a modified manner as a film 22 between the heel of the bullet and the

upper margin of the shell above the powder. It may be applied initially to the inner upper surface or mouth of the shell before the bullet is attached as shown in Figure 4 or it may be initially applied to the heel of the bullet before attachment within the shell as shown in Figure 5.

The most suitable sealing compound which has been found for this purpose is lacquer but there are other sealing compounds having similar properties which may be used. It is possible to use any of the quick drying oils dissolved in a suitable solvent; shellac dissolved in alcohol; or any of the condensation products dissolved in a suitable thinner. Any sealing compound which in the dry or oxidized state is resistant to solvent action of gum oils and greases may be used without departing from the concept of this invention.

20 One suitable formula for a sealing material is as follows:

|                   | Per cent<br>by weight |     |
|-------------------|-----------------------|-----|
| Nitrocellulose    | 13                    |     |
| 25 Gum            | 6                     | 90  |
| Dibutyl phthalate | 4                     |     |
| Butyl acetate     | 26                    |     |
| Ethyl acetate     | 10                    |     |
| Butanol           | 10                    |     |
| 30 Toluene        | 31                    | 95  |
|                   |                       | 100 |

Other lacquers, consisting essentially of nitrocellulose which have been rendered soluble by suitable solvents and to which have been added gums, plasticizers and oils may be used.

Having described my invention, I claim:

1. A cartridge, comprising, a shell, powder and a priming mixture in said shell, a bullet protruding from the shell, and a film of oil proof material disposed between the bullet and shell.

2. A cartridge, comprising, a shell, powder and a priming mixture in said shell, a bullet protruding from the shell, and a film of nitrocellulose lacquer disposed between the bullet and shell.

3. A cartridge, comprising, a shell, powder and a priming mixture in said shell, a bullet protruding from the shell, and a film of drying oil disposed between the bullet and shell.

4. A cartridge, comprising, shell, powder, bullet, said bullet and shell clinched together and a seal disposed at the crevice formed by said clinched connection.

5. In a cartridge, including the shell, powder in said shell and bullet attached in said shell, a film of oil proof sealing material disposed between the adjacent surfaces of said bullet and shell for sealing the jointure.

6. In a center-fire cartridge including a shell, powder in said shell, a bullet attached to said shell and a priming cup secured in the base of said shell, a sealing material disposed about said priming cup for sealing the same

against the entrance of oil or moisture to the powder and priming mixture.

7. In a cartridge, a shell, powder in said shell, a bullet attached in said shell, a priming cup and a seal applied at the joints of the shell and bullet and about the priming cup, said seal composed of nitrocellulose lacquer.

8. A center-fire ball cartridge having a lacquer sealing the joint of the shell and ball, and joint of priming cup in the base of the shell.

9. In a cartridge, a shell, powder in said shell, a bullet attached in said shell, and an adhesive coating of oil and waterproof material applied between the bullet and shell for sealing the cartridge between these parts.

In witness whereof, I hereunto subscribe my name.

GEORGE H. JACOBS.

85

90

95

100

105

110

115

120

125

130